

Aug. 10, 1965

M. A. M. BAKKER ETAL  
PLATINUM COATED MOLYBDENUM GRID HAVING AN  
INTERMEDIATE LAYER OF NICKEL  
Filed May 26, 1961

3,200,284



INVENTOR  
MARTINUS A.M. BAKKER.  
JOHANNES CH. DURAN.  
BY  
*Frank R. Jepson*  
AGENT

# United States Patent Office

3,200,284  
Patented Aug. 10, 1965

1

3,200,284  
PLATINUM COATED MOLYBDENUM GRID HAVING AN INTERMEDIATE LAYER OF NICKEL  
Martinus Antonius Maria Bakker and Johannes Christiaan Duran, both of Emmasingel, Eindhoven, Netherlands, assignors to North American Philips Company, Inc., New York, N.Y., a corporation of Delaware  
Filed May 26, 1961, Ser. No. 112,816  
Claims priority, application Netherlands, July 26, 1960, 254,219  
2 Claims. (Cl. 313—348)

The invention relates to a method of coating by electro-deposition a grid manufactured from molybdenum for electric discharge tubes so that during the whole life of the tube the platinum layer adheres satisfactorily and remains completely intact.

It is known that a platinum layer is capable of keeping the primary grid emission very low, which is of particular importance in transmitting tubes in which the grids often assume a very high temperature.

When a grid consisting of molybdenum wire in its definite shape is coated by electro-deposition with a platinum layer without using further means, it is found that this layer at a sufficient strength disengages during operation of the discharge tube and finally surrounds the molybdenum wire like a rolled down stocking.

It is known to manufacture grids from an Mo-wire which is previously surrounded by a Pt-cylinder and, after heating in a furnace to 1350° C. is rolled or stretched in a reducing atmosphere to form a thin wire. If desired, the molybdenum core wire may be previously subjected to acid treatment and coated by electro-deposition with a nickel layer so that it is adapted to slide with accurate fit in a Pt-cylinder. The intermediate nickel layer then serves as solder for the platinum outer layer.

It is found that grids manufactured from such platinum-coated wire are subjected to deformation and warping during operation, in which event even breakage of the wires may occur.

It is known that it is not possible to coat a molybdenum grid which has already obtained its definite shape first by electro-deposition with nickel and to provide it then by electro-deposition with a platinum layer, since in this case, after removal of the platinum layer from the electro-plating bath, it bursts open immediately or afterwards upon heating. Many investigations have proved that this is due to the fact that the platinum applied by electro-deposition is very brittle as a result of the absorption of hydrogen inevitably liberated during this process and that great mechanical stresses occur in the platinum layer.

The invention provides a method which renders it possible to apply the platinum layer by electro-deposition after the shaping of a molybdenum grid. The molybdenum grid is first coated with a layer having a rough surface of a metal of the iron group (Fe, Co, Ni) and then it is coated with platinum by electro-deposition. Such a rough intermediate layer may be obtained by applying the metal in the form of oxide which is reduced by heating in a reducing atmosphere.

Now it is found that, as a result of the rough structure of the intermediate layer, the above-mentioned difficulties are completely obviated, since the rough intermediate layer constitutes a mechanical anchorage for the platinum layer which is consequently fixed. During subsequent heating and during operation, the attachment is further improved by relative diffusion of the metals. Now it is found that the platinum layer does not burst during manufacture, while by appropriate choice of the thicknesses of

2

the intermediate layer and of the platinum layer the time required for the diffusion of molybdenum from the core to the platinum surface is longer than the life (5000 hours) of the tube in which the grid is used, even at an operational temperature of about 1200° C. Owing to the initially obtained mechanical anchorage of the platinum layer, the latter adheres to the substratum during the whole life of the tube. The diffusion of platinum in the core also proceeds so slowly that, when use is made of platinum layers of thicknesses of 5 to 10 microns, no bare spots will occur on the grid during the life of the tube. Consequently, the favorable emission properties of the grid are maintained.

The intermediate layer may be applied by immersing the molybdenum grid in a suspension of, for example nickel oxide, by drying and heating in a reducing atmosphere until the oxide is reduced to nickel. The thickness of this intermediate layer is, for example, 0.1 $\mu$ . The grid is now coated by electro-deposition with a platinum layer of, for example, 5 to 10 microns and heated during a few hours at 1200 to 1500° C. If the weight of the intermediate layer does not exceed half that of the platinum layer, it has been found that no unfavorable evaporation of this layer occurs during operation of the discharge tube. A thickness of 0.1 $\mu$  has proved to be very favorable. If desired, the intermediate layer may also be provided by electro-deposition and roughened by sandblasting.

Furthermore, it is found that the intermediate layer prevents the disengagement of the platinum layer as a result of the difference between the expansion coefficients of platinum and molybdenum.

The invention will now be described more fully with reference to the drawing, in which:

FIG. 1 shows a grid according to the invention, and FIG. 2 is a sectional view of a grid wire.  
FIG. 1 shows a grid for transmitting tubes which consists of a plurality of U-shaped molybdenum rods 1 which are held together by means of a ring 2. The grid wire 3 is wound on the rods 1. The rods 1 may have a diameter of 1 mm., the wire 3 may have a thickness of 200 microns. The grid is coated completely with a platinum layer 5 having a thickness of 10 microns which is firmly bonded to the molybdenum core 1 by means of a rough intermediate nickel layer 4 of 0.1 $\mu$ .

What is claimed is:

1. A grid for an electric discharge tube comprising a base of molybdenum, an outer layer of platinum, and an intermediate layer of a metal selected from the group consisting of iron, cobalt, and nickel firmly bonding said platinum layer to said base, said intermediate layer having a thickness less than half that of the platinum layer.
2. A grid for an electric discharge tube comprising a base of molybdenum, an outer layer of platinum having a thickness of about 5 to 10 $\mu$ , and an intermediate layer of nickel firmly bonding said outer platinum layer to said base, said nickel layer having a thickness of about 0.1 $\mu$ .

## References Cited by the Examiner

### UNITED STATES PATENTS

- |           |      |         |           |
|-----------|------|---------|-----------|
| 2,539,096 | 1/51 | Miller  | 313—348   |
| 2,821,496 | 1/58 | Perl    | 313—348 X |
| 2,878,549 | 3/59 | Willner |           |
| 3,164,740 | 1/65 | Moscony | 313—348   |

GEORGE N. WESTBY, Primary Examiner.

RALPH G. NILSON, Examiner.